

Nov. 11, 1941.

S. C. LILLEY

2,262,017

ELASTIC STRAND FOR ELASTIC FABRICS

Filed Nov. 28, 1940

10,

Fig. 1.

10,



10,

Fig. 2.

11,



11,



Fig. 3.

11,



10,

11,

Fig. 4.



10,

Fig. 6.

11,



Fig. 7.

Fig. 8.



Fig. 9.



## UNITED STATES PATENT OFFICE

2,262,017

## ELASTIC STRAND FOR ELASTIC FABRICS

Samuel C. Lilley, Hamden, Conn., assignor, by  
mesne assignments, to United Elastic Corpora-  
tion, Easthampton, Mass., a corporation of  
Massachusetts

Application November 28, 1940, Serial No. 367,491

2 Claims. (Cl. 57—149)

The present invention relates to improvements in elastic strands for elastic fabrics and constitutes an improvement upon the elastic strands disclosed in my U. S. Patents Nos. 2,146,965 and 2,146,966, both dated February 14, 1939.

One of the objects of the present invention is to provide a superior elastic strand for incorporation into elastic fabrics, which strand is provided with a superior coating combining heat-activatable properties with the property of protecting the elastic strand proper from the deleterious effects of air, perspiration, and other skin excretions.

Another object of the present invention is to provide a superior elastic strand for incorporation into elastic fabrics with a coating which will not only discharge the function of adhering covering material to the strand-body, but will, at the same time, shield the said elastic strand-body from the deleterious effects of ultra-violet light and chemically-active washing compounds.

A further object of the present invention is to provide a superior elastic strand having a coating of heat-activatable thermo-plastic material capable of securely adhering covering material to the elastic strand proper and at the same time possessing an elasticity approximating the elasticity of the said strand proper, to thereby avoid a rupture between the strand-body proper and the coating material.

With the above and other objects in view, as will appear to those skilled in the art from the present disclosure, this invention includes all features in the said disclosure which are novel over the prior art.

In the accompanying drawing, in which certain modes of carrying out the present invention are shown for illustrative purposes:

Fig. 1 is a broken view in side elevation of an elastic strand-body suitable for being coated with the thermo-plastic adhesive-forming protective coating of the present invention;

Fig. 2 is a similar view but showing a portion of the strand-body provided with a peripheral coating of polymerized iso-butylene;

Fig. 3 is a view in end elevation of the structure of Fig. 2;

Fig. 4 is a broken view in side elevation showing the elastic strand-body partly coated with polymerized iso-butylene and having a helical wrapping applied thereto;

Fig. 5 is an end view of the structure of Fig. 4;

Fig. 6 is a view corresponding to Fig. 4 but showing the addition thereto of an outer helical wrapping of textile material;

Fig. 7 is an end view of the structure of Fig. 6; Fig. 8 is a broken longitudinal sectional view taken on the line 8—8 of Fig. 6, but on a larger scale; and

5 Fig. 9 is a broken view substantially corresponding to Fig. 8, but showing the covered strand after the substantially-dry adhesive-forming coating of polymerized iso-butylene has been activated by heat to adhere the inner layer of covering strands to the elastic strand-body.

As will be apparent from the following, the present invention contemplates the employment of an elastic strand-body having a coating of thermo-plastic adhesive-forming material composed primarily of polymerized iso-butylene which possesses special advantages when combined as a covering upon strand-bodies of rubber-base material.

In carrying out the present invention, an elastic strand-body 10 is employed which in the particular instance shown is of circular form in cross section, though the cross sectional form may be rectangular or of other suitable cross section, as is well known in the art.

15 20 25 30 35 40 The elastic strand-body 10 above referred to may be made of a wide variety of elastic materials such as vulcanized rubber compounds common in the textile art and preferably having a heat-disintegrating point at a temperature materially above the temperature at which the hereinafter-referred-to thermo-plastic adhesive-forming material will effectively soften. Specific examples of elastic materials from which the strand-body 10 or its equivalent may be formed are so numerous and well known in the art as not to require detailed description herein, save to note that as in the case of practically all rubber-base compounds, the material is subject to oxidation and the disintegrating effects of ultra-violet light, etc.

Around the perimeter of the elastic strand-body 10 is applied a coating 11 of thermo-plastic adhesive-forming material formed mainly or entirely of polymerized iso-butylene which is a saturated member of the group which may be designated as aliphatic iso-olefin polymers.

45 50 55 By way of example, the following may be employed as the thermo-plastic adhesive-forming material in conjunction with the rubber-base elastic strand-bodies.

## Example A

Polymerized iso-butylene dissolved in naphtha, toluol, or other suitable solvents, which may be driven off by mild heat, following the completion

of the application of the polymerized iso-butylene to the strand-body.

*Example B*

Polymerized iso-butylene dispersed in water with or without clay, casein, or other suitable dispersing aids.

*Example C*

|                          | Per cent |
|--------------------------|----------|
| Polymerized iso-butylene | 97       |
| Rosin                    | 3        |

Both of the above dissolved or dispersed in either naphtha or its equivalent, or in an aqueous solution.

*Example D*

|                          | Per cent |
|--------------------------|----------|
| Polymerized iso-butylene | 78       |
| Carbon black             | 22       |

The above may be dissolved or dispersed in naphtha or its equivalent, or in an aqueous dispersion.

The coating 11 of polymerized iso-butylene may be applied to the strand-body 10 in any suitable manner such, for instance, as by immersing the said strand-body in a liquid or semi-liquid bath of the said polymerized iso-butylene.

The polymerized iso-butylene, or compounds thereof, is preferably applied to the strand-body 10 in the form of the coating 14 or its equivalent by depositing on the said strand-body an aqueous dispersion or emulsion of the polymerized iso-butylene. Such aqueous dispersion or emulsion is particularly advantageous inasmuch as its use in processing involves no fire hazard. If desired, however, and as before noted, the polymerized iso-butylene may be dispersed in a suitable solvent such as naphtha.

After the strand-body 10 has had the coating 11 or its equivalent applied to it and after the said coating has been dried to a nonliquid condition, a layer of textile covering material 12 may be applied directly over the thermo-plastic adhesive-forming coating 11, as is shown especially well in Figs. 4 and 5.

Should it be found desirable and in order to insure the ready handling of the coated strands of Figs. 2 and 3 and after the same have been substantially dried, the said strand may be treated with talc or other adhesiveness-reducing material such, for instance, as those described in my prior Patent No. 2,146,966. In this manner and under conditions where necessary, the coated strands may be rendered convenient for passing through covering machines, looms, etc., though in most instances the coating 11 may be rendered sufficiently non-tacky by mild heating.

If desired and as is shown especially well in Figs. 6 and 7, a second layer 13 of covering material may be wrapped over the previously described layer 12 when especially severe specifications are to be met.

The covering materials employed such, for instance, as 12 and 13 may be composed of a wide variety of textile or fibrous materials such, for instance, as cotton, wool, regenerated cellulose, etc., which specific examples are substantially inelastic as compared to the elastic strand-body herein referred to.

The coating 14 of polymerized iso-butylene is usually sufficiently soft to permit the convolutions of the covering material 12 to slightly press into the said coating when the said covering material is applied under tension, as is indicated in Fig. 8.

When the elastic strand-body 10 with its thermoplastic adhesive-forming coating 11 is subjected to heat in conjunction with covering material, such as 12, or the crossing strands of 5 an elastic fabric, the said coating 11 will soften or melt to a sufficient degree to secure a firm grip upon the covering material and firmly anchor the same to the strand-body 10. An exposure of the coating 11 to a temperature of about 215° F. for a period of five minutes is usually adequate to secure the necessary bonding. This time and temperature are substantially those employed in finishing elastic fabrics on so-called "dry can" finishing machines. 15 Lesser heats may be employed over longer periods of time or higher degrees of heat over much briefer periods of time. Within reasonable limits, neither the time nor temperatures are critical.

The heating of the coating of polymerized 20 iso-butylene such as 11 to secure the adhesive properties referred to, may be accomplished before or after the coated strand such as is shown in Figs. 2 and 3, is incorporated into a woven, knitted or netted fabric, either with or without the coverings 12 or 13. In some instances, however, it is preferred to adhere covering material, such as 12, to the strand-body prior to the same being incorporated in a fabric and this may be readily accomplished by passing the coated 25 strand with its covering material through a heated chamber, to thus secure continuous straight-line production.

When the coating 11 or its equivalent composed primarily of polymerized iso-butylene is 30 subjected to heat in conjunction with suitable covering material, such as 12, or the crossing strands in a fabric, not only is the strand-body 10 firmly united to the selected covering material but the polymerized iso-butylene coating remains 35 as a protective coating minimizing or substantially eliminating the oxidizing of the rubber-base strand-body 10 or its equivalent and protecting the same also against the deleterious effects of ultraviolet light and of perspiration and other skin excretions, chemically-active 40 washing compounds, etc.

The strands of the character and in the condition especially well shown in Figs. 2 and 3, may 45 be conveniently stored, shipped and sold at normal temperatures without causing objectionable adhesions between various parts of a strand or of various adjacent strands and still retain their ability to become adhered to a covering material when subjected to suitable degree of heat.

Under other conditions, the elastic strands of 50 the present invention may be marketed with adhered covering material such as 12, instead of being marketed in the substantially naked conditions with merely the coating 11 applied thereto and rendered nonliquid.

The elastic and coated strands of the present 55 invention, like those of my prior patents herein referred to, possess the characteristics of being conveniently adhered to any suitable covering material and, in addition the coating of polymerized iso-butylene serves to an exceptional degree to protect the rubber-base strand-body from the deleterious effects of oxygen, perspiration ultraviolet light, etc.

The invention may be carried out in other specific ways than those herein set forth without departing from the spirit and essential characteristics of the invention, and the present 60 embodiments are, therefore, to be considered in 65 all respects as illustrative and not restrictive.

and all changes coming within the meaning and equivalency range of the appended claims are intended to be embraced therein.

I claim:

1. A new article of manufacture, an elastic strand adapted to be woven or knitted into elastic fabrics and to be adhered to textile covering material by heat, and comprising: an elastic strand-body of rubber-base material having its exterior provided with a nonliquid heat-activatable thermo-plastic adhesive-forming material containing over fifty per cent of polymerized isobutylene and adapted to thermo-plastically adhere the said strand body to textile covering material when heated in conjunction therewith; the said rubber-base strand-body forming the major portion of the cross-sectional area of the strand and the said adhesive-forming material forming a minor portion of the said cross-sectional area thereof and acting as a protective coating for the said strand-body, whereby the said adhesive-forming material serves to shield and protect the said strand-body from the deleterious effects of ultraviolet light and other harmful exterior media.
- 5
2. A covered elastic strand of the type adapted to be woven or knitted into elastic fabrics and comprising: an elastic strand-body of oxidizable material; textile covering material extending around the said strand-body; and an adhesive material formed primarily of polymerized isobutylene and adhering the said strand body to the said covering material and vice versa; the said strand-body forming a major portion of the cross-sectional area of the covered strand as compared to the said adhesive material which forms but a minor portion of the said cross-sectional area and acting as a protective coating for the said strand-body, whereby the said adhesive material serves to shield and protect the said strand-body from the deleterious effects of ultraviolet light and other harmful exterior media.
- 10
- 15
- 20

SAMUEL C. LILLEY.